

## UNITED STATES PATENT OFFICE

2,381,440

HIGH DENSITY COMPRESSIBLE IRON  
POWDER AND PROCESS

Joseph E. Drapeau, Jr., Calumet City, Ill., assignor  
to The Glidden Company, Cleveland, Ohio, a  
corporation of Ohio

No Drawing. Application February 6, 1943,  
Serial No. 474,976

10 Claims. (Cl. 75—28)

This present invention relates to an improved type of iron powder and to the method of making the same.

Iron powder heretofore used for the manufacture of pressed shapes has generally been of relatively low specific gravity. This has been necessary or desirable since such powders are made up of particles of irregular shape having rough surfaces, whereby sufficient green strength is produced on pressing. High density iron powders are not suitable for many purposes since the milling necessary to produce the high density results in particles of nearly spherical shape having smooth surfaces, which on pressing do not give the desired green strength in the product when using practicable pressures. High apparent density, however, is desirable in order to reduce the size of the dies used in the pressing operation, and in order to increase the size and number of products which can be produced by this economical method of fabrication.

It is accordingly an object of the present invention to produce an improved high apparent density iron powder.

Another object is to provide a process for producing an improved iron powder having a relatively high apparent density.

Iron powder as ordinarily produced by reduction of iron oxide has a relatively low apparent density due to the porous and irregular nature of the particles. The grains making up the particles of such a powder are of a poly-crystalline nature which results in so-called slip plane interference in the movement of the solid metal under pressure. It has been found, however, that if a high density powder, the particles of which have a mono-crystalline structure, is first subjected to a flash oxidation to produce a surface oxide film, and this film is then subjected to a low temperature reduction for a short time that the desired objects may be accomplished.

The surface oxidation and reduction results in a new iron powder of high apparent density, the particles of which are of mono-crystalline structure and have an outside surface of a spongy porous nature. The mono-crystalline powder, whether of pure ferrite, or iron containing dissolved or dispersed carbides of granular pearlite lends itself to easier slippage of planes bringing about a marked interlocking of the metal powder during pressing. The porous rough surfaces also assist in the interlocking of the particles. The powder is thus one which produces relatively high green strength on pressing with the advantage of

the high apparent density that would not be possible with an untreated iron powder.

In carrying out the invention porous poly-crystalline iron powder produced by the low temperature reduction of iron oxide may be first treated according to United States Patent No. 2,181,123. The porous material is first subjected to a rather severe milling operation to produce a powder of relatively high apparent density, preferably in a mill of the hammer type. This milling reduces the powder particles to approximately spherical shape having smooth surfaces. The milled powder is then subjected to a heat treatment in a reducing atmosphere, or under other non-oxidizing conditions at a temperature at which normal grain growth occurs to convert the poly-crystalline material to the mono-crystalline state. As mentioned in Patent No. 2,181,123, the temperature of this heat treatment will be in the range of 900 to 1650° F.

The mono-crystalline material is then subjected to a short oxidation with air or in air with steam to produce a surface oxidation, whereby the powder becomes dark gray or reddish in color. The amount of oxidation is not great, and the oxide film may only be five or six molecules in thickness. Since a relatively high apparent density is desired the amount of oxidation will not be such that the apparent density of the final powder is less than desired. The partially oxidized material is then reduced with hydrogen, CO or other suitable non-carbonizing reducing material at a temperature low enough to prevent sintering, preferably at about 600° C. This reduction will take place in a very short time. The material thus produced is then cooled under non-oxidizing conditions, given a light tumbling operation and screened. The particles of the material so produced have spongy surfaces of pure ferrite since the surface treatment removes any carbides which may have been originally present in the surface.

Alternatively the conversion from the poly-crystalline state to the mono-crystalline state may be accomplished after the oxidation step, by having the conditions for the reducing action such that grain growth occurs.

The powder thus produced shows a decided improvement over an iron powder of the same chemical analysis and with a mono-crystalline structure, but having smooth surfaced ball-like particles. The powder so produced has an improved green strength and also sinters more rapidly than the untreated powder. The pressed and

sintered product is thus of greater strength. The advantages of high apparent density in the molding operation, however, are retained. An apparent density of from 2.3 to 2.6 is desirable but heretofore such a powder did not produce the desired green strength. The powders produced by the present invention may have such an apparent density, are highly compressible and produce high green strength and rapid sintering pressed products.

It is to be understood that it is within the spirit of the present invention to use as a starting material any iron powder having a relatively high apparent density, and bringing about a roughening of the surface by a surface oxidation followed by reduction, it being kept in mind that if such starting material is poly-crystalline in nature, conversion to the mono-crystalline state will be effected.

The temperature of the heat treatment of the iron powder is preferably above 1000° F. but below the point at which sintering takes place. The maximum is about 1650° F. with a minimum of 900° F. At or above the recrystallization point there is a change from alpha iron, a body centered cubic crystal, to gamma iron, a face centered cubic crystal.

I claim:

1. An iron powder composed of particles of mono-crystalline structure and having thin, porous, spongy surfaces of substantially uniform thickness.

2. An iron powder having an apparent density of from 2.3 to 2.6 and composed of particles of mono-crystalline structure and having thin, porous, spongy surfaces of substantially uniform thickness.

3. An iron powder characterized by having a relatively high apparent density composed of particles of approximately spherical shape of mono-crystalline structure, and having thin, porous, spongy surfaces of substantially uniform thickness.

4. An iron powder composed of particles of mono-crystalline structure having cores containing dissolved carbides and thin, porous, spongy surfaces of pure ferrite iron of substantially uniform thickness.

5. The process of producing an improved iron powder which comprises subjecting an iron powder of relatively high density composed of particles of mono-crystalline structure to a surface oxidation and then to a reducing treatment to reduce iron thus oxidized at a temperature insufficient to cause substantial sintering.

6. The process which comprises subjecting an iron powder composed of substantially spherical particles of mono-crystalline structure and having smooth surfaces first to a surface oxidation, and then to a reducing treatment sufficient to reduce the thus oxidized iron at a temperature insufficient to cause substantial sintering.

7. The process of producing an improved iron powder which comprises subjecting an iron powder to a surface oxidizing treatment, then to a reducing treatment to reduce the iron thus oxidized at a temperature insufficient to cause substantial sintering, said process being further characterized in that the starting material is polycrystalline and the powder is subjected to a treatment to convert the same to mono-crystalline structure at some stage in the process.

8. The process of producing an improved iron powder which comprises converting a powder composed of particles having a polycrystalline structure to particles of mono-crystalline structure, surface oxidizing the mono-crystalline particles and then reducing the thus oxidized surface film at a temperature insufficient to cause substantial sintering.

9. The process of improving iron powder having a polycrystalline structure and relatively low apparent density and composed of irregularly shaped particles which comprises first subjecting such a powder to a milling operation to produce a powder of relatively high apparent density, the particles of which are approximately spherical in shape and have smooth surfaces, subjecting the thus milled powder to a heat treatment to develop a mono-crystalline structure, surface oxidizing the mono-crystalline material, and then reducing the surface oxide film at a temperature insufficient to produce substantial sintering.

10. The process of improving iron powder having a polycrystalline structure and low apparent density and composed of irregularly shaped particles, which comprises subjecting such a powder to a milling operation to produce a powder of relatively high apparent density, the particles of which are of approximately spherical shape and have smooth surfaces, surface oxidizing the particles, subjecting the surface oxidized material to a heat treatment under reducing conditions to reduce the surface oxide film and to convert the polycrystalline material to monocrystalline, the temperature being insufficient to cause substantial sintering.

JOSEPH E. DRAPEAU, JR.